

## UNITED STATES PATENT OFFICE

ADOLF FRY, OF ESSEN, GERMANY, ASSIGNOR TO FRIED. KRUPP AKTIENGESELLSCHAFT,  
OF ESSEN-ON-THE-RUHR, GERMANY

## LOW CARBON STEEL

No Drawing. Application filed December 16, 1927, Serial No. 240,649, and in Germany August 27, 1928.

This application is a continuation in part of my application Serial No. 149,280, filed November 18, 1926.

Articles made of low carbon steel suffer from the drawback, in particular when in aged condition, of becoming brittle, when exposed to the effect of liquids, vapors and gases which may cause a feeble reaction, for instance hot caustic soda solution of 45 per cent, alkaline boiler feed water or ammonia gases. My invention has for its object to obviate this drawback.

According to the invention this object is obtained by employing for the manufacture of said articles a low carbon steel of a content of carbon up to 0.4 per cent and in which the substances tending to segregate between the grain boundaries, such as oxygen, oxygen compounds, sulphur, carbon etc., are prevented from doing so.

The reason why the said drawback of becoming brittle is obviated by preventing these substances from segregating between the grain boundaries, may be as follows:

The substances generally present in low carbon steel, such as oxygen, oxygen compounds, sulphur, carbon etc., have the tendency to segregate between the grain boundaries, where they form either an intermediate layer separating the individual grains, or small nests, which in itself decreases the tenacity of the material to some extent. Now, when such a steel, in particular when in aged or tensioned condition, is exposed for instance to the effect of a hot caustic soda solution of 45 per cent, the solution advances along the grain boundaries and dissolves the oxygen out of them, whereby the coherence prevailing between the individual grains is lessened. This process results in the great decrease of the tenacity—measured by a bending test of a notched bar of the steel—which is feared in the art as the so-called solution-brittleness and appears after a relatively short time. A similar phenomenon arises when the steel is exposed to the effect of vapors or gases. If, for example, the effect is produced by hot hydrogen gas at about 500° C. and under high pressure, the hydrogen penetrating along the grain bound-

aries generates volatile hydrocarbon compounds with the carbon present between the grain boundaries in the form of pearlite, said compounds washing the carbon away from the grain boundaries and causing small cavities to be produced in the texture. This phenomenon likewise results in the steel becoming brittle very quickly. A similar brittleness is caused when sulphur which may exist in the grain boundaries, is dissolved by the effect of vapors or gases.

The result common to all these cases is that a brittleness of the steel is developed, instead of the said originally prevailing normal tenacity, and that this brittleness is caused by removing substances from the grain boundaries of the steel only when the articles have come into use. If, however, the substances mentioned are prevented from segregating between the grain boundaries, or removed therefrom from the beginning, that is before the articles are used, for instance in the manner hereinafter proposed, a much more intimate coherence of the grains will prevail, as this coherence is not disturbed by any noxious intermediate layer or nests. Consequently, the possibility that the liquids, vapors and gases in consideration will penetrate along the grain boundaries into the steel and thus lessen the coherence of the grains is very much reduced or totally removed. Hence, the originally prevailing tenacity "of the bent notched bar" cannot be substantially decreased, or decreased at all, even after a long action of said liquids, vapors and gases upon the steel.

In the case of steel which has already become solid and wherein, therefore, the substances mentioned have already segregated between the grain boundaries, then by heating the steel at a temperature above about 650° C. and subsequently quenching it with or without reheating up to a temperature not exceeding 750° C., the said substances are made to enter into solid solution with the steel and are held in this condition. In particular, the carbon may be changed, by annealing the steel at about 730° C., into the form of grained carbide and be removed in this manner from the grain boundaries.

Now, when the said substances are most finely divided by quenching from the state of solid solution or the carbon is in the condition of grained carbide, so that the grain boundaries are free from them, there is practically no possibility that the liquids, vapors and gases will be capable of dissolving said substances out of the texture when acting upon the steel, and thus of causing the brittleness.

It may be left undecided how far the explanations made hereinbefore will stand firm in detail against scientific investigation. In every case, however, it clearly appeared from exact experiments, that test pieces of a steel treated in the indicated way, showed their original tenacity after having been exposed for a long time to the attack of hot caustic soda solution of 45 per cent. Other test pieces of the same composition, but not subjected to a previous treatment according to my invention, were destroyed in a short time by cracks, after having been exposed in a similar manner to the attack of the soda solution.

What I claim as my invention and desire to secure by Letters Patent, is:—

1. Articles which must be capable of withstanding the corrosive effect of mildly corrosive liquids, gases, and vapors, characterized by the fact that they are composed of a steel containing an amount of carbon not more than 0.4%, which steel has been quenched from a temperature of 650° to 35 950° C.

2. Articles which must be capable of withstanding the corrosive effect of mildly corrosive liquids, gases, and vapors, characterized by the fact that they are composed of a low carbon steel which has been quenched from a temperature of 650° to 950° C. and subsequently drawn at a temperature not exceeding 750° C.

3. Articles which must be capable of withstanding the corrosive effect of mildly corrosive liquids, gases, and vapors, characterized by the fact that they are made of a low carbon steel which has been heated to a temperature of about 730° C.

50 The foregoing specification signed at Cologne, Germany, this 30th day of November, 1927.

ADOLF FRY.